

April 9, 1935.

A. MEISSNER

1,997,263

METHOD OF MANUFACTURING THIN DIELECTRIC MATERIALS FOR HIGH POTENTIAL WORK

Filed July 3, 1929



INVENTOR  
ALEXANDER MEISSNER

BY *H. E. Brown*  
ATTORNEY

## UNITED STATES PATENT OFFICE

1,997,263

## METHOD OF MANUFACTURING THIN DI-ELECTRIC MATERIALS FOR HIGH POTENTIAL WORK

Alexander Meissner, Berlin, Germany, assignor to Telefunkens Gesellschaft für Drahtlose Telegraphie m. b. H., Berlin, Germany, a corporation of Germany

Application July 3, 1929, Serial No. 375,891  
In Germany July 4, 1928

5 Claims. (Cl. 204—31)

The present invention relates generally to an improved method of manufacturing insulation materials.

More specifically the present invention is directed toward a system of manufacturing relatively thin insulation materials by subjecting the insulation material while in a molten or soft state during its manufacture to the action of an electrical field.

10 Considerable experimentation has shown that insulation materials can be improved a great deal by subjecting the material during its manufacture, that is, while it is still in a soft or liquid state to a powerful electrical field and allowing 15 the material to solidify or consolidate in the presence of such an electrical field. The electrical field may be obtained, for instance, by applying electrodes on one or both faces of the insulation material while it is solidified. Across the 20 two electrodes a potential ranging between 1 and 10,000 volts is applied depending upon the thickness of the dielectric material. Of course, these values given are here included simply for illustration and it is to be distinctly understood that 25 any voltage commensurate with the thickness of the dielectric material may be employed. While I do not desire to hold myself to any particular explanation of the phenomena involved I believe that the reason why dielectrics treated in accordance 30 with my invention are greatly improved is because if the dielectric material is still soft or liquid, that is, not yet solidified then by the action of such a strong electrical field very strong forces are brought to act upon the insulating or 35 dielectric material. One possible explanation of this is that by the action of such a field and the electrodes all the air bubbles or cavities and impurities in the electric substance are forced away from the electrodes. That this is so is shown 40 by the fact that if a dielectric substance or insulation material has been treated in the manner set forth above and if it is fractured or cut and the fracture examined it will be found that a considerably greater density and concentration 45 and more uniform disposition of the constituent particles of the dielectric are produced at the electrodes. In the case of thin layers or coats it will be found sufficient to apply only a unilateral field. I have also found that in the case of thick 50 layers concentration or compacting of the material in the vicinity of the electrodes may be insured most suitably while the layers are being rolled or pressed as the case may be. For this purpose the rolling cylinders or pressing members 55 are furnished with potential at one or both sides.

The single figure in the drawing shows by way of example one method by which my invention may be practiced. In said figure a mold is shown comprising a matrix 1 and a patrinx 2 with metallic coats 3 and 4. To the metallic coats 3 and 4 there is applied a potential of the desired intensity by way of supply leads 5 and 6. In the drawing 7 represents in a general way the mass of insulation material which is to be molded, pressed, or rolled as the case may be.

If thin layers are manufactured and must be made serviceable also for relatively high potentials then a plurality of thin layers manufactured as here directed are superposed or else they may be made by inserting a metal foil or a metalized deposit on the material and using this metal foil or deposit as an electrode for the next layer to be produced. It should here be noted that the present method of constructing insulating materials is particularly useful in the manufacture of insulated wires. In such cases the insulation while still in a molten state and while hardening on the wire may be subjected to the action of a powerful electrical field with the result that the insulation material is pressed with great force against the metal surface of the wire. Throughout this specification and claims which are to follow I intend to use the term "insulation material" generically and intend that it cover such materials as bakelite, glass, porcelain, rubber, etc.

I claim:

1. The method of manufacturing dielectric material which comprises subjecting the material while in a molten state to the action of a uni-directional electrostatic field and subjecting the material to pressure while being cooled within said uni-directional electrostatic field.

2. The method of manufacturing dielectric material which comprises subjecting the material while in a molten state to the action of a uni-directional electrostatic field and subjecting the material to pressure between pressing members having the uni-directional electrostatic field applied to said members while said material cools.

3. The step in the method of making electric insulation material which comprises subjecting the material while in a molten state to the action of an electric field in a uni-directional manner and allowing the material to cool and harden while under the influence of said electric field so as to arrange the polar axes of the molecule complexes parallel with each other.

5 10 15

20 25

30

40

45

50

55

4. The steps in the method of making electric  
insulation material which comprises subjecting  
the material while in a molten state to the action  
of a uni-directional electric field so as to ar-  
5 range the polar axes of the molecule complexes  
parallel with each other and allowing the mate-  
rial to solidify while under the action of the  
electric field.

5. The method of making a solid body, com-  
prising insulation materials having molecule  
complexes which include the steps of heating the  
body to a liquid state, then chilling the same  
within the confines of a uni-directional electric  
field until converted again into a solid state. 5

ALEXANDER MEISSNER.